

## UNITED STATES PATENT OFFICE

2,250,470

## MANGANESE ALLOY

Reginald S. Dean and Clarence T. Anderson, Salt Lake City, Utah, assignors to Chicago Development Company, Chicago, Ill., a corporation of Illinois

No Drawing. Application September 23, 1940,  
Serial No. 357,922

6 Claims. (CL. 75—134)

This invention relates to non-ferrous alloys having a high degree of corrosion resistance, especially with respect to brines and dilute acids. It relates particularly to such alloys wherein manganese is present as a major constituent and is especially concerned with alloys of manganese, copper, nickel and chromium which may be hardened by heat treatment.

The alloys of the present invention fall within the range of manganese from 30% to 90%, nickel from 1% to 35%, chromium from 1% to 20%, and the balance substantially all copper, the copper comprising at least 5%. A particularly preferred range is about 40% to about 50% manganese, about 33% to about 40% copper, about 5% to about 15% nickel, and the balance comprising about 5% to about 15% chromium.

The alloys within the composition ranges above specified are ductile and corrosion resistant when quenched from temperatures ranging from about 900 degrees C. to 1000 degrees C. They may be hardened by heat treatment after quenching, a preferred form of this treatment comprising heating the quenched alloy to a temperature of approximately 425 degrees C. for a period of about 12 hours. It will be understood, of course, that the amount of hardening produced will depend upon the particular composition of the alloy as well as upon the exact mode of heat treatment.

For example, if the composition of the alloys, with the exception of the chromium content, in other words, the proportions of manganese, copper and nickel, fall within the range disclosed in our copending application, Serial No. 300,798, filed October 23, 1939, then the hardening will not be greatly affected by the addition of up to about 10% of chromium. With higher percentages of chromium in this group of alloys, there is a tendency for the alloy to become brittle. The addition of chromium to alloys within this range increases their corrosion resistance.

The addition of chromium to alloys of manganese, copper and nickel within the broader composition range specified hereinabove, but outside the range of hardenable alloys described in our aforementioned application, Serial No. 300,798, makes such alloys readily susceptible to hardening by heat treatment. The hardness which is obtainable by heat treatment varies, among other things, with the chromium content, being relatively slight with 1% chromium, reaching a substantially maximum hardness at approximately 10% to 12% chromium, and showing brittleness at about 20% chromium.

The following examples are illustrative of alloys falling within the scope of the present invention. It will be understood that these are merely representative and that the full scope of the invention is not in any wise to be limited to the examples given, but is to be construed in accordance with the claims.

## Example I

10 An alloy was prepared by melting together 45 parts by weight of electrolytic manganese, 36 parts by weight of electrolytic copper, 9 parts by weight of electrolytic nickel and 10 parts by weight of electrolytic chromium. The resulting alloy may be fabricated hot or cold. Its tensile strength, after quenching from 1000 degrees C., was approximately 75,000 pounds per square inch and it had a hardness of zero as measured on the Rockwell C scale. After heating at 425 degrees C. for 12 hours, the hardness on the Rockwell C scale was 49. In the hardened condition, the alloy was exceptionally tough. It was highly corrosion resistant to salt water and dilute acids in both the soft and hardened condition.

## Example II

20 An alloy was made by melting together 77 parts by weight of electrolytic manganese, 9 parts by weight of electrolytic copper, 5 parts by weight of electrolytic nickel, and 9 parts by weight of electrolytic chromium. The resulting alloy, as quenched from 1000 degrees C., had a tensile strength of 60,000 pounds per square inch and a hardness of —14 as measured on the Rockwell C scale. On reheating the alloy at a temperature of 425 degrees C. for 12 hours, its hardness, on the Rockwell C scale, increased to 42 and its tensile strength increased to 180,000 pounds per square inch. In both the hard and soft states, the alloy was corrosion resistant.

## Example III

30 An alloy was made by melting together 50 parts by weight of electrolytic manganese, 40 parts by weight of electrolytic copper, 9 parts by weight of electrolytic nickel, and 1 part by weight of electrolytic chromium. The resulting alloy, as quenched from 100 degrees C., had a tensile strength of 59,000 pounds per square inch and a Rockwell C hardness of —15. On heating the alloy at 425 degrees C. for 12 hours, its tensile strength increased to 85,000 pounds per square inch and its hardness to Rockwell C —4.

40 In addition to the mechanical and corrosion resistant properties of the alloys of the present

invention which have been pointed out hereinabove, we have also studied their electrical resistance and temperature coefficients of expansion. In general, the electrical resistance of these alloys is high, varying from approximately 100 microhms/cm.<sup>3</sup> to about 140 microhms/cm.<sup>3</sup> The coefficient of expansion of these alloys is also relatively high, varying from about 15 to about 25. The higher coefficients of expansion are found in those of the alloys which contain the minimum amount of chromium and whose composition, except for the chromium content, falls closely within the range of manganese, copper and nickel set forth in our copending application Serial No. 303,006, filed November 6, 1939.

In the preparation of the alloys of the present invention, we have found it to be particularly advantageous to employ substantially pure metals. In the case of manganese, we prefer particularly to employ electrolytic manganese having a purity of 99.9+. Manganese derived from other sources but of substantially equal purity can also be used with good results. When the amount of chromium is relatively small, the so-called pure chromium of commerce may be utilized. However, when chromium approaches the maximum percentage as specified in accordance with the present invention, we find it distinctly advantageous to use electrolytic chromium.

It will be understood that the invention encompasses alloys of the type described hereinabove wherein minor percentages of other elements are added but where the fundamental characteristics and properties of our alloys are not adversely affected.

What we claim as new and desire to protect by Letters Patent of the United States is:

1. A hardenable alloy, having good corrosion resistant characteristics, containing manganese from 30% to 90%, nickel from 1% to 35%, chromium from 1% to 20%, and the balance substantially all copper, the copper comprising at least 5%.

2. An alloy containing from 1% to 20% chromium, from 5% to 56.5% copper, from 30% to 90% manganese, and the balance, to total substantially 100%, being from 7% to 22.5% nickel, the manganese being present in amounts of at least about four times that of the nickel.

3. A quenched and reheated alloy, having high hardness and good corrosion resistant properties, containing manganese from 30% to 90%, nickel from 1% to 35%, chromium from 1% to 20%, and the balance substantially all copper, the copper comprising at least 5%.

4. An alloy containing about 40% to about 50% manganese, about 33% to about 40% copper, about 5% to about 15% nickel, and the balance comprising about 5% to about 15% chromium.

5. An alloy containing approximately 45% manganese, approximately 36% copper, approximately 9% nickel, and the balance chromium.

6. A quenched and reheated alloy, having high hardness and good corrosion resistant characteristics, containing the following elements in substantially the stated proportions:

|           | Per cent |
|-----------|----------|
| Manganese | 40 to 50 |
| Copper    | 33 to 40 |
| Nickel    | 5 to 15  |
| Chromium  | 5 to 15  |

30

REGINALD S. DEAN.  
CLARENCE T. ANDERSON.

35